

## UNITED STATES PATENT OFFICE

DANIEL MANSON SUTHERLAND, JR., OF MORRISVILLE, PENNSYLVANIA

## ROT-PROOF FIBER PRODUCT

No Drawing.

Application filed September 10, 1930. Serial No. 481,077.

My invention relates to rot-proof fiber products and their manufacture, such as building board made out of woody fiber. I aim to produce a board of superior biological resistance, and to make possible the manufacture of such board in a simple and inexpensive manner. The invention is of special advantage in connection with waterproof board, and I have hereinafter explained it with special reference to the manufacture of board of that character.

In practice, fiber board is made from fiber pulp, consisting of wood fiber mixed and suspended in a large volume of water. This pulp is brought into a layer of proper thickness, which is partly freed of its water and then dried, either with or without pressure. In making waterproof board according to my preferred process, I include in the pulp, or add to it, a waterproofing agent or material, and also a toxic agent or material, which will destroy or render harmless the organisms that deteriorate the fiber,—whether termites or the like, or rot-producing organisms in the strict sense. The agents or materials thus incorporated with the pulp are used in such quantity or form that when the water of the pulp is removed, a sufficient amount of waterproofing and toxic materials will remain interspersed amongst the fibers in the board. In other words, the interstices amongst the interlaced fibers are charged (though preferably not filled) with the waterproofing material and the toxic material, which last is combined with the waterproofing material more or less uniformly, and the fibers are practically covered with these materials and cemented together by them.

As a waterproofing agent may be used any substance or material having this property that can be incorporated with the pulp so as to be properly distributed in the fiber board, such as water-soluble rosin size, rosin-wax size, or wax size. Many materials commonly known as waterproofing agents can be incor-

porated in fiber pulp to water-proof the board made therefrom.

A great variety of well-known toxic reagents or materials can be used, including the many well-known toxic-metal salts, as well as coal tar creosote, etc. In general, I prefer insoluble toxic salts as the toxic material in the board, and particularly the toxic salts containing copper, zinc, arsenic, or mercury. Such salts (as well as creosote) are, in general, compatible with rosin size, and sufficiently powerful and inexpensive to be commercially feasible. Being insoluble in water, they readily remain with the fiber when the water of the pulp is drained away; and are not liable to soak or wash out of the board if exposed to the weather, or otherwise wet. On the other hand, they are poisonous to termites attacking the board; and they are dissolved by the cellulose-decomposing acid secreted by rot-producing organisms, which by means of this acid break down the cellulose to starch, which they can assimilate. The fine particles of such insoluble salts mix readily with the pulp, and are distributed more or less uniformly and embedded in the waterproofing material in the final fiber board.

A pulp suitable for my purpose may be prepared according to the following formula:

|                                   | Pounds |
|-----------------------------------|--------|
| Fiber                             | 1000   |
| Rosin size (bone dry basis)       | 20     |
| Zinc meta-arsenate, $Zn(AsO_2)_2$ | 3      |
| Water, about                      | 50000  |

The soluble rosin size and the powdered toxic metal salt are thoroughly mixed with a small amount of water, sufficient to dissolve the rosin size readily, and this mixture is stirred in with the pulp. The pulp is then run into a pressing mold ("wet machine") with provisions for draining off the water, or otherwise formed into a "raw" pulp sheet freed of most of the water. This raw sheet

may then be pressed between heated drier plates, and thus converted into strong, coherent, waterproof board, consisting of the interlaced and compressed fibers and the 5 rosin (not resoluble in water), which cements the fibers together and practically covers them. The insoluble particles of toxic salt are dispersed throughout the rosin and embedded therein, as already mentioned.

10 In the formula above given, 50 lbs. of creosote may be substituted for the zinc meta-arsenate, with equally good toxic effect. The creosote has a strong odor which may render the board objectionable for some purposes, though specially desirable as a lining 15 for moth closets and the like.

Wood has heretofore been rot-proofed by "secondary" impregnation with various substances, and it has been proposed to treat 20 fiber board in the same way. Such impregnation, however, is subject to serious practical drawbacks:

(1) Only liquids or reagents in solution can be introduced into the pores of the material in this way. Water-soluble toxic 25 reagents, however, are easily washed or soaked out of the board.

(2) To impregnate a board with an insoluble toxic material, a two-step process is 30 necessary: i. e., the board must first be impregnated with a solution of one reagent, and then with a solution of another reagent which will react with the first to precipitate the desired insoluble material in the pores of 35 the board.

(3) The pores can never be completely 40 filled with any solid introduced in solution,—whether by a one-stage or two-stage process,—since the solvent water has to be driven out.

(4) It is difficult or impossible to effectively rot-proof a thoroughly waterproofed board by impregnation, since its pores are already filled or clogged with the water- 45 proof material.

All of these difficulties and disadvantages of secondary impregnation are overcome by incorporating the rot-proofing and waterproofing agents or materials in the pulp, as 50 described above: no special operation whatever is really required, since the pulp is always thoroughly stirred or agitated before formation into a sheet, as a matter of ordinary manufacturing practice.

55 Having thus described my invention, I claim:

1. A rot and water-proof and termite-proof fiber board, comprising interlaced fibers having their interstices charged with 60 a waterproofing material and a toxic agent combined therewith.

2. A rot and water-proof and termite-proof fiber board, comprising interlaced fibers having their interstices charged with 65 a waterproofing material, and particles of

an acid-soluble, water-insoluble toxic-metal salt embedded in said waterproofing material.

3. A rot and water and termite-proof fiber board, comprising interlaced fibers having 70 their interstices charged with a waterproofing material, and particles of zinc meta-arsenate imbedded in said waterproofing material.

In testimony whereof, I have hereunto 75 signed my name at Trenton, New Jersey, this 27 day of August, 1930.

DANIEL MANSON SUTHERLAND, Jr.

80

85

90

95

100

105

110

115